

July 5, 1955

S. SOBEL

2,712,190

IRIDESCENT MATERIAL AND PRODUCT

Filed May 29, 1953

Fig. 1.



Fig. 2.



Fig. 3.



Fig. 4.

INVENTOR.  
SOL SOBEL  
BY *Karen Sobel*

ATTORNEY

## IRIDESCENT MATERIAL AND PRODUCT

Sol Sobel, Plainfield, N. J., assignor to Rainbo-Cel, Inc., Perth Amboy, N. J., a corporation of New Jersey

Application May 29, 1953, Serial No. 358,307

16 Claims. (Cl. 41—10)

This invention relates to iridescent products and is concerned more particularly with the provision of plastics products having an iridescent appearance.

It has been proposed heretofore to impart an iridescent effect to the surface of wrapping material having a Celluloid base or to films of cellulose derivatives or to cellulose papers made transparent by means of resin or similar materials by applying to such surface a bismuth or antimony compound, and then applying thereover a film of strongly diluted solutions of resins or film formers, e. g. a film of liquid Celluloid. Such materials, although satisfactory as wrapping sheets are not satisfactory when shredded into flakes and an attempt is made to incorporate them into plastics carrier bodies, to make decorative articles such as costume jewelry, buckles, buttons, studs and the like, since they quickly lose their iridescent effect. Also, the degree of iridescence of the wrapping material alone is markedly inferior and lacking in quality. Such a teaching is exemplified, for example, by the British patent to Wickel 294,463, of April 18, 1928.

It has also been proposed to form ornamental objects from plastics by incorporating therein light reflecting particles, such as pearl essence, metal foils, particles of powder, metallic salts, etc. Further, these bodies have been cut in a specific manner, e. g. so that the light reflecting particles are oriented in a direction generally parallel to the long axis of the body. However, all such products do not exhibit iridescence, e. g. the display of rainbow colors on a surface due to thin films, which cause interference of light rays, but rather such heretofore known products have been referred to as being pearly, nacreous, silky, chatoyant, etc., i. e. lusters arising from layers of reflecting surfaces. Such a teaching is exemplified by the British patent to Meyer 548,834, of April 23, 1941.

It has further been proposed, in an attempt to obtain iridescent effects in plastics products, to heterogeneously and indiscriminately incorporate cubes, blocks, discs, or portions of differently pigmented plastics into a plastic mass of cellulose organic derivative base material on steam-heated kneading rolls. It is important to note that in such prior art suggestions the structure of the flake was obtained by mixing a colloidal suspension of pearl essence, mica dust, metallic salts or powders, etc., with a plasticizer and then homogenizing the mixture with a plastics mass on kneading rolls, the cooled product thereafter being shredded into flakes. Such flakes do not exhibit any marked degree of iridescence when subsequently incorporated into a plastics body. Such a teaching is contained in the U. S. patent to Conklin, 2,154,438, issued on April 18, 1939.

I have now determined that if a polyfilmed flake is incorporated into a plastics base material, wherein the flake includes at least two metallic films, an iridescent product may be formed which will exhibit the same degree of iridescence as exhibited by the flake itself.

It is, therefore, one object of this invention to provide an iridescent material which shall have a greater decorative effect than similar products heretofore known. It

is another object of this invention to provide an iridescent product containing such material which shall be capable of greater adaptability than other such products as heretofore known and which shall, therefore, be capable of wider use than heretofore possible. It is a further objective of this invention to provide products for the costume jewelry industry which shall have an enhanced eye appeal. Other advantages and objects of my invention will appear from the description thereof hereinafter following:

5 The invention is illustrated in the accompanying drawings, forming part of this specification, and in which:

Figure 1 is a cross-sectional view of the iridescent material of my invention,

Figure 2 is a cross-sectional view of another embodiment of the iridescent material of the invention,

Figure 3 is an elevational view of a part of the product of the invention, and

Figure 4 is an elevational view of another embodiment of the product of the invention.

My invention contemplates the provision of iridescent material in the form of transparent or light-transmissive flat laminae which may be shredded into flakes. The product of the invention has dispersed throughout its mass, a single flake, or heterogeneous fragments, or the like.

As used hereinafter, the term "plastics" is used as both the singular and the plural, and is intended to include that group of synthetic or natural polymeric materials which can be shaped when soft and hardened afterwards.

30 Also, as used hereinafter, the term "light transmissive" is intended to include both transparent and translucent material.

Referring to Figure 1, the iridescent material has a base layer 1, of plastics, and has a first outer layer 2, also of plastics material. Alternatively, the base layer may have two first outer layers, one on each side of the base layer. Optionally, a second outer layer 3, also of plastics material may be used, however, such second outer layer may be omitted, if desired. Interposed between the base layer

40 1 and the first outer layer 2; and on the surface of the layer 2, or between the layers 2 and 3, are thin metallic films 4 and 5, of the same or different materials. It is necessary that the outer film 5 be light transmissive, however the inner film 4 may be opaque, if desired. The several layers may consist of the same or of different plastics material. In Figure 2 I have shown a further embodiment wherein four metallic films 4, 5, 8 and 9 are employed, interspersed among layers 1, 2, 3, 6 and 7. As indicated above, the outermost layer 7 may be omitted.

50 The thin metallic films consist of metal and/or metallic compounds. If a metal compound is used, preferably the salt, then the surface of each layer is polished with such metallic compound. For example, bismuth oxychloride or other halogen compounds of bismuth or com-

55 pounds of other metals may be used. At least the outermost metallic film of the flake must be light transmissive. Also, a pure metal may be used, and it may be electro-deposited on the plastics layers or put on by high vacuum deposition.

60 The iridescent effect is obtained by the interference of light reflected from the front and the back of the thin film, and through the plastic layers and the metallic films therebetween. The thickness of the film determines the color attributed to it; thus, as the thickness of the film increases, its apparent color changes analogous to that of the well-known Newton rings. Therefore, the extremely thin films of the first order are white, yellow or red, while those that are thicker exhibit apparent colors that are red, orange, greenish-blue, etc. Where the laminated material has a plurality of such layers, the thickness may be varied from layer to layer to produce a variety of iridescent effects.

Any of the plastics may be used as the layer material, such as the thermoplastic and thermosetting plastics, natural and synthetic resins, etc. For example, of the thermoplastic plastics, the cellulose ethers such as ethyl cellulose, methyl cellulose, benzyl cellulose or cellulose acetate, nitrocellulose, polystyrene, superpolyamides, acrylate polymers, styrol resins and the like, or combinations thereof, may be used. Of the thermosetting plastics, phenols or phenol-aldehydes such as phenol formaldehyde or unsaturated polyester or alkyd, allyl esters and the like, resorcinols, furans, ureas, silicones, epoxies or combinations thereof may be used.

Figure 3 shows a form of the use of the iridescent material of the invention. The iridescent material 10, in various shapes of flakes, such as discs, thin sheets, triangles, tape, etc., is dispersed through a carrier medium 11, shown as a rod. It is to be understood, however, that the carrier medium may assume any desired physical shape, e. g. umbrella frames, optical frames, etc., or may be supported on any other body. In Figure 4, the flake material 12 is embedded in a transparent carrier body 13 in the form of a sphere, which may form a bead for necklaces, bracelets, etc.

The product may be formed by casting or molding, i. e. injection compression, extrusion, etc. The abovementioned thermosetting plastics are primarily useful as the carrier body in the case of castings and compression molding, while extruded products are preferably formed with the thermoplastic materials. The flake can be employed in all usual methods of handling thermoplastics, i. e. injection molding, laminating, etc.

The following specific examples are illustrative of the present invention, but are not to be construed as being limitative of the scope thereof.

#### Example I

A cellulose acetate film, approximately .002" thick, was placed on a smooth surface. The film was then polished by rubbing both sides with a fine cloth which was dusted with bismuth oxychloride, for such time and with such pressure, so as to deposit on the surface a transparent highly reflectant metallic film. Then, wiping with a clean cloth, the excess powder was removed. A solution of nitrocellulose was prepared and dissolved in amy1 and butyl acetate with a viscosity of approximately .50 poise at 77° F., and the film was coated therewith by immersing it in the solution. The film was then withdrawn vertically at approximately three inches of movement per minute. After the coating had dried and adhered to the cellulose acetate film, it was polished on both sides with bismuth oxychloride and wiped with a clean cloth to remove any excess powder. The now iridescent material was then shredded to a desirable size.

#### Example II

A cellulose nitrate film, approximately .002" thick, was placed on a smooth surface. The film was then polished by rubbing on both sides with a fine cloth which was dusted with bismuth oxyiodide for such time and with such pressure so as to deposit on the surface a highly reflectant metallic film of a reddish tint. Then, wiping with a clean cloth, the excess powder was removed. A solution of styrene polymer dissolved in styrene monomer was prepared with a viscosity of approximately .50 poise at 77° F., and the film was coated therewith by immersing it in the solution. The film was then withdrawn vertically at approximately three inches of movement per minute. After the coating had dried, and adhered to the cellulose nitrate film, it was polished with bismuth oxyiodide on both sides, and wiped as above described. The now iridescent material was then shredded to a desirable size.

#### Example III

A polyvinylidene chloride film was placed on a smooth surface. The sheet was then polished as described in

Example I, supra. A solution of cellulose acetate dissolved in methyl Cellosolve acetate with a viscosity of approximately .50 poise at 77° F., was prepared and the film was coated therewith by immersion. The film was then withdrawn and allowed to dry as in the above examples. It was then polished again, as described in Example I. A solution of vinyl butyral was then prepared and dissolved in a mixture of butyl and methyl alcohol at a viscosity of approximately 80 seconds on a  $\frac{1}{2}$  Ford Cup at 77° F., and the coated film was immersed in this solution and withdrawn at the rate of two inches of movement per minute. When it was dry, it was again repolished and wiped as described in Example I. The iridescent material was then shredded into flakes.

#### Example IV

A film of aluminum was deposited by high vacuum deposition onto a low volatile regenerated cellulose film. A solution of methyl methacrylate dissolved in its monomer was prepared at a viscosity of approximately .50 poise at 77° F. The regenerated cellulose film was then immersed in the acrylic solution and withdrawn as in Example I. When this coating was dry, it was polished, wiped and shredded as described in Example I.

#### Example V

A film of gold was deposited by high vacuum deposition onto a low volatile polyvinyl alcohol film. A solution of ethyl cellulose was prepared at a viscosity of approximately .50 poise at 77° F. The polyvinyl alcohol film was immersed in ethyl cellulose solution and withdrawn as in Example I. When this coating was dry it was polished, wiped and shredded as described in Example I.

#### Example VI

A film of silver was deposited by high vacuum deposition onto a low volatile nylon film. A solution of cellulose acetate butyrate was prepared at a viscosity of approximately .50 poise at 77° F. The nylon film was immersed in cellulose acetate butyrate solution and withdrawn as in Example I. When this coating was dry it was polished, wiped and shredded as described in Example I.

In the last three examples, the metallic film may also have been provided by electroplating or flame spraying, etc.

The iridescent material or flake, produced as described in the above examples may be incorporated in a plastics carrier body to form a desired product. Any plastics material may be used for the carrier body, such as polyesters, phenolics, ureas, melanines, casein, cellulosics, acrylics, vinyls, etc. The following examples are illustrative of the formation of a product embodying the iridescent material.

#### Example VII

An allyl polyester resin (e. g. "Kriston") was catalyzed with 1% by weight of benzoyl peroxide and heated at about 167° F. for about one to two hours until thickening occurred. Such a plastics material exhibits sufficiently high viscosity so that before thickening occurred a plurality of iridescent fragments, such as those produced in Example I above, was introduced and the mixture was stirred until a uniform distribution of flake was obtained. The mixture was then cast into a desired shape, i. e. a rod. Curing takes place after about two hours.

#### Example VIII

Unsaturated polyester in styrene (e. g. "Paraplex") was catalyzed with 5% by weight of benzoyl peroxide and before gelation occurs, or just at the moment of gelation, iridescent fragments such as described in Example I were introduced, however the flakes had an outer layer of phenol formaldehyde. Curing was obtained at 200 degrees F.

*Example IX*

A properly catalyzed phenolic resin (e. g. "Catabond") was poured into a mold of a desired configuration. The flakes were then added and the mixture in the mold was thoroughly stirred to obtain uniform distribution. Curing was obtained at about 175° F.

The hereinbefore described specific examples of this invention have all illustrated how iridescent flakes and products may be formed. However, as previously indicated, the scope of the invention is not limited to the specific metals and plastics mentioned. Thus, for example, any plastics material may be substituted for the layers or the carrier body material mentioned above. Also, any metal or form thereof, may be used in any manner, known per se, for forming the film.

During the manufacture of the product, care must be taken that the plastics material of the iridescent flake and the plastics material of the carrier body are not, at the temperature employed and during the period of contact, while the carrier material is soft or fluid, soluble one in the other; since otherwise the sharply defined boundary between the dispersed medium and the carrier body would be destroyed. Therefore, for each type of iridescent flake it is necessary to select a plastics carrier body of a material compatible therewith, so that the temperature requirements of the carrier body are not in excess of the temperature limitations of the iridescent material, so that there is no solvent or chemical reaction between the two. Furthermore, it is important, especially in the case of casting of the thermosetting plastics and monomers, that the fragments or media to be dispersed are floated into the carrier material while the latter is in such a state of viscosity that a uniform distribution of the dispersed medium throughout the carrier body is possible without settlement thereof during the curing or hardening of the carrier body.

For molding thermosetting materials, or for molding and extruding thermoplastic materials, the iridescent particles may be incorporated with the molding compound in any suitable manner; for example, on kneading rolls, or in dry mixing with the molding compound, or where practical, the iridescent particles may be introduced into the monomer.

The transparent carrier body may be backed up, where desired, by an opaque surface, e. g. in the form of a black plastics or an applied opaque surface. While the specific examples deal with a carrier body and with flake layers of transparent plastics material, other light-transmissive materials, such as translucent plastics or vitreous materials may of course also be used. Also, of the layers of the flake, the base or first layer may be of opaque material as long as the outer layer is light transmissive.

The product of my invention is characterized by a high eye appeal throughout, substantially all of the loosely dispersed fragments or flakes generally participating in the iridescent effect, thus creating a sparkling iridescence not heretofore obtained. As illustrative of the failure of the prior teaching to provide iridescent products comparable to that taught by this invention, the following comparison was made:

*Example X*

A sheet of cellulose acetate film, approximately .002" thick, was polished on one side by rubbing with a fine cloth which was dusted with bismuth oxychloride for such time and with such pressure so as to deposit on the surface of the sheet a highly reflectant metallic film. The excess powder was then removed by wiping with a clean cloth. The coated layer was then immersed in a nitrocellulose solution, and withdrawn as described in Example I, supra. Upon drying, this material was found to exhibit an iridescence. Such material is exemplified in the prior art by the above-mentioned patent to Wickel. The coated film was then cut in two and one portion was re-polished and the excess removed as described in Example

I, supra. Both portions were then immersed into a beaker of styrene monomer. Upon observance it was noted that the portion of the material which represented the prior known teachings lost its iridescent property and merely became light transmissive, whereas the portion of the material which had the two metallic films, according to the teachings of my invention exhibited the same degree of iridescence as it had formerly.

Other arrangements of the layers and films of the flake than shown in the drawings and modifications in the product containing the flakes will be readily apparent to those skilled in the art and are intended to be included within the scope of the invention.

This application is a continuation-in-part of my prior filed applications Serial Numbers 165,398 and 165,399, both filed on June 1, 1950, now abandoned.

What I claim is:

1. An iridescent product consisting of a carrier body at least partially composed of light transmissive plastics material, having dispersed therethrough a discrete medium of iridescent material in the form of a flake, said flake being characterized as comprising a base layer of a solid material presenting an upper and a lower surface, at least one of said surfaces having thereon a minimum of two metallic films one of which is light transmissive and an interposed layer of a light transmissive plastics material therebetween, the layers and films being so arranged as to have a light transmissive layer and a light transmissive film juxtaposed on a surface of the flake, the substances of the layers, films and carrier body being so chosen that they do not become interfused during manufacture.

2. The iridescent product of claim 1 wherein the flake has a second light transmissive plastics material layer over the outer metallic film.

3. An iridescent product consisting of a carrier body at least partially composed of light transmissive plastics material, having dispersed therethrough a discrete medium of iridescent material in the form of a flake, said flake being characterized as comprising a base layer of a solid material presenting an upper and a lower surface, both of said surfaces having thereon a minimum of two metallic films one of which is light transmissive and an interposed layer of a light transmissive plastics material therebetween, the layers and films being so arranged as to have a light transmissive layer and a light transmissive film juxtaposed on a surface of the flake, the substances of the layers, films and carrier body being so chosen that they do not become interfused during manufacture.

4. The iridescent product of claim 3 wherein the flake has a light transmissive plastics material layer over each of said outer metallic films.

5. The iridescent product of claim 1 wherein the base layer is of a plastics material.

6. The iridescent product of claim 1 wherein the two metallic films encompassing the interposed layer are both light transmissive.

7. The iridescent product of claim 1 wherein the base layer is of light transmissive plastics material.

8. An iridescent flake comprising a base layer of a solid material and presenting an upper and a lower surface, at least one of said surfaces having thereon a minimum of two metallic films one of which is light transmissive and an interposed layer of a light transmissive plastics material therebetween, the layers and films being so arranged as to have a light transmissive layer and a light transmissive film juxtaposed on a surface of the flake, the substances of the layers, films and carrier body being so chosen that they do not become interfused during manufacture.

9. The iridescent flake of claim 8 wherein the flake has a second light transmissive plastics material layer over the outer metallic film.

10. An iridescent flake comprising a base layer of a solid material and presenting an upper and a lower sur-

face, both of said surfaces having thereon a minimum of two metallic films one of which is light transmissive and an interposed layer of a light transmissive plastics material therebetween, the layers and films being so arranged as to have a light transmissive layer and a light transmissive film juxtaposed on a surface of the flake, the substances of the layers, films, and carrier body being so chosen that they do not become interfused during manufacture.

11. The iridescent flake of claim 10 wherein the flake has a second light transmissive plastics material layer over the outer metallic films.

12. The iridescent flake of claim 8 wherein the solid material of the base layer is plastics material.

13. The iridescent flake of claim 12 wherein the two

metallic films encompassing the interposed layer are both light transmissive.

14. The iridescent flake of claim 13 wherein the base layer is light transmissive.

15. The iridescent product of claim 1 wherein the plastics material of the layers is a thermosetting plastic.

16. The iridescent flake of claim 8 wherein the plastics material of the layers is a thermosetting plastic.

References Cited in the file of this patent

FOREIGN PATENTS

|         |               |                |
|---------|---------------|----------------|
| 281,100 | Great Britain | Dec. 1, 1927   |
| 294,463 | Great Britain | Sept. 18, 1929 |
| 479,508 | Great Britain | of 1938        |
| 548,834 | Great Britain | Oct. 27, 1942  |